

# UNITED STATES PATENT OFFICE.

JUAN DE M. TERREFORTE, OF NEW YORK, N. Y., ASSIGNOR TO HIMSELF  
AND ANTONIO M. MOLINA, OF SAME PLACE.

## ART OF PRINTING AND MOUNTING PHOTOGRAPHIC PICTURES.

SPECIFICATION forming part of Letters Patent No. 295,688, dated March 25, 1884.

Application filed June 27, 1883. (No specimens.)

*To all whom it may concern:*

Be it known that I, JUAN DE M. TERREFORTE, of the city, county, and State of New York, have invented certain new and useful 5 Improvements in the Art of Printing and Mounting Photographic Pictures, of which the following is a full, clear, and exact description.

In carrying my invention into practice, I 10 provide a solution, which I call "solution No. 1," composed of refined gelatine, fifteen parts; distilled water, one hundred parts; chloride of ammonium, one part. The above are to be mixed under a gentle heat and filtered through 15 muslin. I also prepare a solution, "No. 2," composed of refined gelatine, ten parts; distilled water, eighty parts. The above are to be mixed under a gentle heat, and to the mixture I then add a solution of nitrate of silver, 20 made by dissolving four parts of crystallized nitrate of silver in ten parts of distilled water. The two solutions or mixtures Nos. 1 and 2 are then mixed together, and I thus produce a sensitive emulsion of chloride of silver ready 25 for use, which is to be carefully preserved from access of light.

Upon a well-cleaned glass plate I form a film 30 of plain collodion, which is allowed to dry, and upon the collodion film I then pour a quantity of said sensitive emulsion, sufficient evenly to coat the collodion film. I then allow the plate to dry. In this manner I produce a sensitive plate ready for the usual photographic printing process. If it is desired to increase 35 the sensibility of the plate, I now submit the sensitive coating to the fumes of ammonia in the same way that ordinary photographic sensitized paper is treated. I print the picture in the ordinary manner, by placing a negative 40 in contact with the sensitive surface of my prepared plate, and subject the same to the action of light. I then develop, tone, fix, and wash the picture in substantially the same manner that ordinary photographic pictures are treated, using chloride of gold for 45 toning and hyposulphite of soda for the fixing, and then wash the picture in water for half an hour, more or less. When the picture is dry, it presents the beautiful appearance of 50 a finished transparency on glass; and in this condition it may, if desired, be colored by the

application thereto of suitable pigments in the ordinary manner. The picture is now transferred from the glass and mounted upon paper in the following manner: I cover the 55 face of a sheet of paper with a thin solution of gelatine, which I press upon the finished picture on the glass and leave the paper to dry thereupon under pressure. I then apply a knife under the edges of the paper and strip 60 the paper, and with it the attached picture and collodion, from the glass. The picture thus produced and mounted on the paper presents a beautiful appearance, having a smooth and glossy face, caused by the collodion film. The 65 picture may then be trimmed and further mounted upon suitable stiff card-board. If desired, the picture may be made to resemble those taken upon porcelain plates. This I effect by mounting my picture in the first instance upon polished hard white cartridge-paper.

Pictures made in accordance with my invention are more durable and have a finer appearance than the ordinary pictures that are 75 printed on paper, which latter, owing to the action of the air, light, and chemicals upon the fiber of the paper, are apt to turn yellow and lose their beauty in a short time.

Among the advantages of my improvement 80 are the following: The picture is printed and finished upon a pellicle or non-fibrous body; hence the finest details of light and shadow in the negative are reproduced in the print with fidelity and brilliancy. Any desired special 85 tint or color may be given to the whole picture by dipping the same in a suitable tinting solution prior to mounting it upon paper; or, if desired, a tinted paper may be used on which to mount the picture, which will, in some 90 cases, give a pleasing appearance to the picture. Another important advantage of my improvement is a saving of nitrate of silver. For my process I only require five per cent. of silver in the sensitizing-mixture, whereas 95 the ordinary photographic-printing process, in which albumen paper is used, requires fifteen per cent. of silver in the sensitizing-bath. Thus I am enabled by my process to produce the finest quality of pictures, while using only 100 one-third of the quantity of the silver ordinarily consumed in making paper prints.

I do not abandon or dedicate to the public any patentable feature set forth herein and not hereinafter claimed, but reserve the right to claim the same, either in a reissue of any patent that may be granted upon this application or in other applications for Letters Patent that I may make.

Having thus described my invention, what I claim as new, and desire to secure by Letters Patent, is—

The method herein described of taking and mounting photographic pictures, which consists in preparing upon glass or other suitable surface a film of dry collodion, then spreading upon the collodion film a sensitive coating of gelatinous or albuminous emulsion con-

taining nitrate of silver, then drying the same, then printing and developing the picture in the ordinary manner upon said sensitized coating, then attaching paper to the picture by applying paper that is faced or coated with plain moist gelatine or albumen to the picture upon the glass, then allowing the paper to dry under pressure in contact with the picture, and then stripping the paper, and with it the picture, from the glass, all substantially as herein described.

JUAN DE M. TERREFORTE.

Witnesses:

EDGAR TATE,  
ALFRED H. DAVIS.